

# UNITED STATES PATENT OFFICE.

ALBERT FREY, OF BASEL, SWITZERLAND, ASSIGNOR TO THE HOFFMANN-LA ROCHE CHEMICAL WORKS, OF NEW YORK, N. Y., A CORPORATION OF NEW YORK.

## PROCESS FOR THE MANUFACTURE OF METAL PYROPHOSPHATE CASEIN COMPOUNDS COLLOIDALLY SOLUBLE IN DILUTE ALKALINE SOLUTIONS.

1,381,295.

Specification of Letters Patent. Patented June 14, 1921.

No Drawing.

Application filed March 20, 1920. Serial No. 367,465.

To all whom it may concern:

Be it known that I, ALBERT FREY, a citizen of Switzerland, and a resident of Basel, Switzerland, have invented certain new and useful Improvements in Processes for the Manufacture of Metal Pyrophosphate Casein Compounds Colloidally Soluble in Dilute Alkaline Solutions, of which the following is a specification.

10 My invention relates to a new process for the manufacture of metal pyrophosphate casein compounds colloidally soluble in dilute alkaline solutions, which consists in dissolving casein in alkali pyrophosphate and adding another metal salt to this solution.

Compounds which contain albumin, phosphoric acid and metals have already been used for therapeutic purposes. In view of the use they are put to, such products should 20 be quite easily soluble in alkali, because in such case only their absorption in the intestinal alkaline juice is assured. The metal phosphoric acid albumin compounds known heretofore meet these requirements not at all, 25 or only partially.

According to the processes known heretofore relating to the manufacture of metal phosphoric acid albumin compounds, casein is for instance dissolved in alkali and the 30 alkaline solution treated with sodium phosphate and solutions of metal salts. In one instance it has been proposed to completely saturate the acid valences of casein by taking it up in an excess of alkali or alkaline earth, and to combine the metaphosphoric acid with the albumin molecule by adding metaphosphoric acid to the alkaline solution. Another process already known describes in a similar manner the manufacture 35 of tricalcium phosphate albumin compounds. Both these processes have the disadvantage of yielding products which are not soluble in alkali. In order to render the products more easily soluble in alkali, it has been

40 recommended to use greatly diluted solutions, but this is unfavorable in practice. It has further been proposed to use pyrophosphoric acid and its salts for the manufacture of calcium- and iron-phosphoric acid albumin compounds, soluble in alkali; here 45 too special emphasis is laid upon the addition of free alkali for obtaining the desired products. Besides their inefficient solubility in alkali the products heretofore known

have the disadvantage of containing but 55 little phosphoric acid, which no doubt is due to the addition of free alkali when combining the phosphoric acid with the albumin molecule.

In the new process, casein, without having previously been dissolved in alkali, is taken up in a solution of alkali pyrophosphate and another metal salt added to the solution. The resulting product meets all requirements. By the simple means of dissolving in alkali pyrophosphate the combination of phosphoric acid with the albumin molecule is brought about at the same time. The mixture shows an acid reaction after the addition of the metal salt, by which fact the 60 transformation distinguishes itself from the processes known heretofore, which latter employ an alkaline solution. The metal phosphoric acid casein compounds contain a great deal of metal pyrophosphate and are 65 entirely soluble in alkali. The process of the present invention has the advantage of 70 allowing the use of concentrated solutions.

The metal pyrophosphate casein compounds colloidally soluble in dilute alkaline 75 solutions are to be used for therapeutic purposes.

### Example 1.

66 parts of casein are dissolved in a solution of 112 parts of crystallized sodium pyrophosphate and 800 parts of water and, while stirring, 156 parts of a four times normal solution of calcium chlorid are added to the mixture. The new compound is precipitated by adding alcohol. After having 80 been washed it is dried at 50° C. The product contains 50% of calcium pyrophosphate and its solutions in sodium bicarbonate and diluted solution of sodium carbonate are 85 stable.

### Example 2.

6.6 parts of casein are dissolved in a solution of 11.2 parts of sodium pyrophosphate and 120 parts of water and to this 19.5 parts 90 of a 23% solution of ferric-chlorid are added, while stirring. The compound obtained is precipitated with alcohol, washed and dried at 50° C. It contains 50% of ferric pyrophosphate. The product is easily soluble in 95 alkali; the solutions are stable.

I claim:

1. As a new article of manufacture the

22  
metal pyrophosphate casein compounds col-  
loidally soluble in dilute alkaline solutions,  
which are entirely soluble in alkali; the so-  
lutions of this compound in sodium bicar-  
5 bonate and diluted solutions of sodium car-  
bonate are stable.

2. The process for the manufacture of  
metal pyrophosphate casein compounds col-  
loidally soluble in dilute alkaline solutions  
10 which comprises dissolving casein in alkali

pyrophosphate adding a metal salt to this  
solution and precipitating the compound  
thus produced.

In witness whereof I have hereunto set  
my hand.

ALBERT FREY.

Witnesses:

HEINRICH KUBLI,  
HUBERT RAUCH.